

## UNITED STATES PATENT OFFICE

2,273,562

## PHOTOGRAPHIC EMULSION

Edward P. Davey and Edward B. Knott, Wealdstone, England, assignors to Eastman Kodak Company, Rochester, N. Y., a corporation of New Jersey

No Drawing. Application July 25, 1946, Serial No. 347,489. In Great Britain August 29, 1939

9 Claims. (Cl. 95—7)

This invention relates to improvements in photographic emulsions such as gelatino silver halide emulsions.

Various substances are known to have a stabilizing effect on photographic emulsions when incorporated therein, that is, they prevent any undue increase in fog on keeping or after incubation of the emulsion. Among the compounds previously proposed for this purpose are the 2-amino-4-hydroxy pyrimidines and the 2-mercaptop-4-hydroxy pyrimidines, including certain substitution derivatives thereof, and their salts. All of these compounds possess only two polar groups, which are dissimilar, and have only one amino, hydroxyl or mercapto group.

We have now found that photographic emulsions may be stabilized by adding thereto with or without sensitizing dyes a small proportion of a pyrimidine compound containing two or more amino or hydroxyl groups. Certain of these compounds have been found to possess in addition a pronounced anti-fogging action by reducing the initial veil of the emulsion without any substantial reduction of the sensitivity.

An object of our invention, therefore, is to provide photographic emulsions of enhanced stability. Another object is to provide stabilized photographic emulsions having low initial fog or veil. Other objects will appear hereinafter.

Pyrimidine has the formula



and the names of the compounds given in this specification are in accordance with the numbering shown.

The compounds used in practising our invention may also carry additional polar or non-polar substituents. The non-polar substituents may be alkyl, aryl, aralkyl, arylene or the like whilst the polar substituents are preferably additional amino or hydroxyl groups. Compounds containing three or four amino and/or hydroxyl groups are especially valuable. The 2 position in the pyrimidine ring is preferably occupied and usually the 4 and/or 5 positions.

We have found that pyrimidines containing amino or hydroxyl groups in the 2 and 5 positions are especially useful since they are valuable anti-fogging agents in addition to being stabilizers. Such 2:5 pyrimidines may also contain additional non-polar substituents such as those defined above, the preferred compounds having

in addition an amino or hydroxyl group in the 4 position.

The invention includes the use of tautomeric forms of the above compounds and also their salts.

The following are examples of pyrimidines which may be used according to our invention either in the form shown or as their salts, for example as their sulphates. It is to be understood that many of the compounds mentioned below may exist in various tautomeric forms which are considered to be within the scope of the present invention. Thus, most of the names given are of enolic compounds but these may also exist in the keto form.

- A. 2:4-dihydroxy-6-amino pyrimidine
- B. 2:6-diamino-4-hydroxy pyrimidine
- C. 2:4:6-triamino pyrimidine
- D. 2-amino-4:6-dihydroxy pyrimidine
- E. 2:6-dihydroxy-4-methyl pyrimidine
- F. 2:4-dihydroxy-5:6-diamino pyrimidine
- G. 2:5:6-triamino-4-hydroxy pyrimidine
- H. 2:4:5:6-tetramino pyrimidine
- I. 2:5-diamino-4:6-dihydroxy pyrimidine
- J. 2:4:6-trihydroxy-5-amino pyrimidine
- K. 2:4:5:6-tetrahydroxy pyrimidine
- L. 2:6-dihydroxy-4-methyl-5-amino pyrimidine
- M. 1-methyl-2-hydroxy-4-keto-5:6-diamino pyrimidine
- N. 1:3-dimethyl-2:4-diketo-5:6-diamino pyrimidine
- O. 2-hydroxy-4:6-dimethyl-5-amino pyrimidine

Methods of preparation of the above and other related compounds will be apparent to persons skilled in the art, using the various processes which have been described in the literature or by obvious modifications of such processes. The following list gives references to methods which may be used for the preparation of the examples given herein, the compounds being identified by the reference letters previously given.

- A & F: Berichte, 33, 1373 or J. A. C. S., 1933, 55, 1667.
- B & G: As above, but using guanidine instead of urea.
- C & H: Berichte, 1904, 39, 4544.
- D & I: Berichte, 1893, 26(B), 2551.
- K: Annalen, 1838, 26, 276.
- E: Annalen, 1885, 229, 5.
- L: Am. Chem. J., 1908, 40, 19.
- O: Modification of the above.
- J: By conversion of barbituric acid into violuric acid followed by reduction with sodium hydrosulphite.

In practice, it has been found suitable to add only a very small amount of the pyrimidine compound to the emulsion at any suitable stage of its preparation but preferably either immediately before coating or during the digestion stage after washing. The amount varies, but on an average concentrations of 0.01 to 0.05 gram per litre of photographic emulsion are suitable but more may be used according to the nature of the emulsion. Generally speaking, the maximum amount of pyrimidine compound necessary for a quantity of emulsion containing the equivalent of 100 grams of silver nitrate will be of the order of 0.10 gram for negative emulsions or 0.25 gram for positive emulsions. When the pyrimidine is added during the digestion stage less is usually required than when it is added just prior to coating. Also the use of the pyrimidine compounds during the after-ripening process is more controllable, the increase in veil with continued digestion being less than normal and the time of digestion being thus less critical.

The practical application of the method of our invention may be illustrated by the figures given in Tables I-III which show the measurements of fog and speed obtained on photographic emulsions treated according to the invention. The reference letters given in the tables relate to the compounds identified by the same letters in the foregoing list of examples.

The results given in Table I were obtained on a high speed gelatino silver bromide emulsion containing 6% silver iodide, 2.5 litres of this emulsion containing the equivalent of 100 grams of silver nitrate. The pyrimidine compound was added during the after-ripening stage in the manufacture of the emulsion, an aqueous solution of the sulphate being made up and sufficient added to the emulsion to give a concentration of 0.01 gram of pyrimidine compound per litre of emulsion. The resulting emulsion was subsequently colour-sensitized by addition of a cyanine dye giving a maximum spectral sensitivity at 620 m $\mu$  and then coated on to glass plates in the usual manner. In order to obtain a control a portion of the emulsion was colour-sensitized and coated as above but without the addition of any pyrimidine compound.

The effect on the fog of the emulsion was determined by developing samples of the plates, without exposure to light, in a metol hydroquinone developer of the usual type for four minutes at 20° C. and measuring the fog density produced with and without addition of the pyrimidine compound. Further samples of the plates, with and without pyrimidines in the emulsion were then incubated at a temperature of 130° F. for a period of seven days and the fog determined as above. The effect on the speed of the emulsion was determined in an analogous manner by exposing behind a step-wedge for  $1/25$  second to light having the characteristics of average daylight and developing as above. The exposure in metre-candle seconds necessary to produce a silver density of 0.2 above fog on development is given as a comparative measurement of the speeds of the emulsions before and after incubation and in each case with and without addition of pyrimidine compound. The columns headed "Stabilized" give in each case the results obtained on samples containing the compounds identified by the reference letter in the left-hand column, whilst the columns head-

ed "Control" give the results on the samples to which no pyrimidine was added.

Table I

| Ref. | Fog        |         |            |         | Speed      |         |            |         |
|------|------------|---------|------------|---------|------------|---------|------------|---------|
|      | Normal     |         | Incubated  |         | Normal     |         | Incubated  |         |
|      | Stabilized | Control | Stabilized | Control | Stabilized | Control | Stabilized | Control |
| 10   |            |         |            |         |            |         |            |         |
| A    | 0.07       | 0.08    | 0.10       | 0.14    | 370        | 380     | 630        | 630     |
| B    | 0.09       | 0.08    | 0.19       | 0.53    | 501        | 575     | 692        | 427     |
| C    | 0.14       | 0.08    | 0.16       | 0.14    | 638        | 380     | 724        | 630     |
| D    | 0.10       | 0.08    | 0.16       | 0.53    | 692        | 575     | 661        | 427     |
| E    | 0.30       | 0.16    | 0.70       | 1.20    | 724        | 1,090   |            |         |
| F    | 0.08       | 0.08    | 0.09       | 0.14    | 417        | 380     | 870        | 630     |
| G    | 0.10       | 0.08    | 0.14       | 0.14    | 398        | 380     | 400        | 630     |
| H    | 0.07       | 0.08    | 0.10       | 0.14    | 724        | 380     | 630        | 630     |
| I    | 0.07       | 0.08    | 0.08       | 0.14    | 525        | 380     | 1,000      | 630     |
| J    | 0.08       | 0.10    | 0.08       | 0.14    | 525        | 380     | 890        | 630     |
| K    | 0.08       | 0.10    | 0.08       | 0.14    | 479        | 380     | 1,400      | 630     |
| L    | 0.07       | 0.12    | 0.08       | 0.14    | 347        | 380     | 870        | 630     |
| M    | 0.07       | 0.08    | 0.13       | 0.14    | 347        | 380     | 900        | 630     |
| N    | 0.08       | 0.08    | 0.09       | 0.14    | 398        | 380     | 980        | 630     |
| O    | 0.24       | 0.16    | 0.42       | 1.20    | 1,112      | 760     | 1,000      | 630     |

The above results clearly show the usefulness of the compounds of the invention as stabilizers for photographic emulsions. The compounds denoted by the reference letters F to O inclusive are pyrimidines substituted in the 2 and 5 positions by hydroxyl or amino groups and it is apparent that, in addition to acting as stabilizers, these compounds also give a noticeable reduction in initial fog but without the loss of speed which is usually associated with the use of antifogging agents.

In Table II are given the measurements obtained in a similar manner to those of Table I but on a not specially colour sensitized high-speed gelatino-silver bromide emulsion containing about 3% silver iodide, 2 litres of this emulsion containing the equivalent of 100 grams of silver nitrate. The pyrimidine compound in this case was added immediately prior to coating, the sulphates being used. The exposure, development and incubation of the emulsions were carried out in the same manner as described above.

The following measurements were obtained on the emulsion after addition of .01 gram per litre of the compound indicated, the reference letters denoting the same compounds as before and the letter Z indicating the measurements obtained on the control samples.

Table II

| Ref. | Fog    |           | Speed  |           |
|------|--------|-----------|--------|-----------|
|      | Normal | Incubated | Normal | Incubated |
| A    |        |           |        |           |
| F    | 0.08   | 0.18      | 820    | 600       |
| G    | 0.05   | 0.10      | 750    | 550       |
| H    | 0.06   | 0.11      | 700    | 800       |
| Z    | 0.05   | 0.10      | 800    | 870       |
| Z    | 0.08   | 0.20      | 800    | 600       |

The advantages of the compounds of our invention as stabilizers and as anti-foggants are again apparent from the above figures.

In Table III are given the results obtained on a gelatino silver bromide emulsion of moderate speed, containing about 1% silver iodide and the same amount of silver as the emulsion used for the tests in Table II but which had not been colour sensitized, the pyrimidine compound being added as the sulphate during the after-digestion stage in the preparation of the emulsion. These measurements were made in similar manner to those previously described. The following

measurements were obtained on the emulsion after addition of .01 gram per litre of the compound indicated during the after-digestion stage. The letter Z again relates to the control samples.

Table III

| Ref.   | Fog    |           | Speed  |           |
|--------|--------|-----------|--------|-----------|
|        | Normal | Incubated | Normal | Incubated |
| A----- | 0.03   | 0.15      | 380    | 327       |
| F----- | 0.03   | 0.11      | 283    | 300       |
| I----- | 0.03   | 0.13      | 316    | 303       |
| Z----- | 0.03   | 0.22      | 330    | 300       |

Although in the examples given in this specification the pyrimidines have been used in the form of their sulphates these are only given by way of illustration since the compounds may be used in the form of the free base or any other convenient salt. In practice it is convenient to make up a solution of the pyrimidine compound in a suitable solvent and add the requisite proportion of such solution to the emulsion or other medium as required. The sulphates are particularly suitable for this purpose as they are sufficiently soluble in water to enable solutions of appropriate strengths to be prepared. However, other solvents may be used to dissolve the compounds provided they have no deleterious effect on the sensitive emulsion; for example, alcohol may be used.

Instead of incorporating the pyrimidine compounds in the sensitive emulsion layer they may, as an alternative, be incorporated in any other convenient layer of a photographic element. Such layer may be an adjacent layer such as a substratum layer or a supercoat over the emulsion layer, or the compounds may even be incorporated in the support.

It is to be understood that the above examples and methods of procedure are illustrative only and that our invention is to be taken as limited only by the scope of the appended claims.

What we claim as our invention and desire to be secured by Letters Patent of the United States is:

1. A sensitive silver halide photographic emulsion stabilized by the presence therein of a pyrimidine compound containing at least two like polar substituents selected from the group consisting of amino and hydroxyl groups.

2. A photographic silver halide emulsion stabilized by the presence therein of a pyrimidine compound containing at least two like polar substituents, selected from the group consisting of amino and hydroxyl groups, situated in the two and four positions.

3. A photographic silver halide emulsion stabilized by the presence therein of a pyrimidine compound containing at least two like polar substituents, selected from the group consisting of amino and hydroxyl groups, situated in the two and five positions.

4. A photographic silver halide emulsion stabilized by the presence therein of a pyrimidine compound containing at least two like polar substituents, selected from the group consisting of amino and hydroxyl groups, situated in the two and five positions.

5. A photographic silver halide emulsion stabilized by the presence therein of a pyrimidine compound containing at least three polar substituents, selected from the group consisting of amino and hydroxyl groups, situated in the two, four and five positions.

6. A photographic gelatino silver halide emulsion containing as a stabilizer a pyrimidine compound containing at least four polar substituents, selected from the group consisting of amino and hydroxyl groups.

7. A sensitive photographic element comprising a light-sensitive layer and in contact therewith, a layer containing as a stabilizer a pyrimidine compound containing at least two like polar substituents selected from the group consisting of amino and hydroxyl groups.

8. A sensitive photographic element comprising a gelatino-silver halide emulsion layer and in contact therewith, another layer containing a pyrimidine compound containing at least two like polar substituents, selected from the group consisting of amino and hydroxyl groups, situated in the two and five positions.

9. A sensitive photographic element comprising a gelatino-silver halide emulsion layer and in contact therewith another layer containing a pyrimidine compound containing at least three polar substituents, selected from the group consisting of amino and hydroxyl groups, situated in the two, four and five positions.

EDWARD P. DAVEY.  
EDWARD B. KNOTT.